

## UNITED STATES PATENT OFFICE

2,046,750

## PRESSURE INVERSION PROCESS OF MAKING HARD BOARD PRODUCTS

William H. Mason and Charles H. Westphalen,  
Laurel, Miss., assignors to Masonite Corporation, Laurel, Miss., a corporation of Delaware

No Drawing. Application April 12, 1934,  
Serial No. 720,247

17 Claims. (Cl. 92—61)

The present invention relates to a process of making hard fiber products, and is an improvement on the patent to Mason No. 1,663,505, granted March 20th, 1928. The invention has for 5 an object to enable the production of an improved hard board or other fiber product practically free from surface defects, by providing an improved mode of hot pressing, herein called a pressure inversion process. In accordance with the improved pressure inversion process, extra high pressure is initially applied for a short interval to a fiber body, or wet lap containing considerable water, as for example, more than 25% of water, usually more than 50% of water. Thereafter the pressure is reduced and the hot pressure operation is carried on under such reduced pressure, except that for the higher density boards the pressure may be raised again when the moisture content has been sufficiently reduced.

A further object is to save drying time and the expense of heat-drying out of water, which by the present process is pressed out more effectively by the high initial pressure. Other objects will 25 appear in the following description of illustrative procedure, it being understood that the invention is not limited to the particular procedures described herein, but is as broad as the claims.

The fiber to be used is made from growths, 30 such as trees, grasses, canes, corn-stalks, and the like containing ligno-cellulose fiber. The raw materials may be shredded or ground or fibrated in other ways, so long as plenty of the non-cellulose content is retained in the fiber with the cellulose to secure effective coalescing or bonding with high wet strength of the hot pressed board. Explosion by high pressure steam of wood chips, followed by partial refining, as by beating, is the preferred mode of fiber preparation. Made of 35 such ligno-cellulose fiber, the product, as a board, has high wet strength and appears to be bonded by the natural non-cellulose material in the fiber. A small percentage, as 2%, of petroleumatum or other waterproofness-enhancing agent 40 is preferably incorporated. Extraneous binders and fillers are permissible, but not essential.

The wet lap, usually containing about 60% of water is introduced in a heated platen press with wire mesh between a face thereof, preferably 45 the lower face, and a press platen.

To secure best and most uniform results the press should have provision for rapid control of heating steam to the platens, controls for rapidly moving the platens toward and away from one 50 another, and in the case of a multiple platen

press such as is preferably used, provision may be made for equalizing the pressure on the individual boards.

The pressure initially applied is extra high and is adapted to press out substantially the maximum 5 quantity of expressible liquid water, and to secure extra high surface qualities in such skin-like portion of the board as is being consolidated at the smooth surface farthest from the wire mesh, through which mesh the expressed water escapes. The escaping water carries with it 10 solubles, and the resulting reduction of solubles remaining in the board is of advantage because, with too great soluble content, there is increased 15 tendency to production of surface defects. Some saving in expense and reduction in drying time 20 are obtained by the efficient expression of liquid water.

After a short interval at the extra-high initial 25 pressure the water outflow is over, and the pressure, preferably without ever being completely released, is reduced to a lower pressure adapted in combination with the effect produced by the higher initial pressure to yield a board of the desired density. About one minute at the extra 30 high pressure and one-half minute time for effecting the reduction have given good results.

In making a board of 1-1.05 specific gravity, for example, the extra high initial pressure may be about 400-500 pounds per square inch, and 35 reduced after about one minute to about 100-125 pounds per square inch and drying completed in about 10 minutes or less for a board  $\frac{1}{8}$ " thick. Lower or higher pressures will reduce or raise 40 the density. It was noted, for example, that with an initial pressure of 200 pounds per square inch, followed by a reduced pressure of 60 pounds per square inch, a board of .9 specific gravity was produced, and drying completed in about 20 minutes for a board  $\frac{1}{4}$ " thick. These figures are 45 illustrative only, and there may be considerable variation on either side.

Use of the ordinary temperatures heretofore 50 available for manufacture of hard board from wet lap as, for example, temperatures in the general neighborhood of 350°-400° F. requires times about as stated above, but a material saving in time can be obtained by heating the platens and the boards to an apparently critical high temperature over about 430° F. and preferably about 55 450°-550° F., which has been found to bring out a new plasticity not available at temperatures below about 400° F. and thus to make the best and hardest board.

This pressure reduction, following the initial 55

application of extra high pressure, is observed, when using a 21 platen hydraulic press, making 20 boards at a time, to be accompanied by a temporary expansion of the boards, which expansion 5 may be up to about 10 or 15% of the finished thickness of board, and is particularly noticeable if the pressure is reduced rather rapidly, as may be done if desired. By this expansion the remaining water content in the board is apparently redistributed throughout the mass and largely withdrawn from the preferably smooth finish surface furthest away from the wire mesh, thereby minimizing likelihood of producing defects at such surface.

15 The drying is continued at the lower pressure, preferably without change, the pressure being followed up as shrinkage takes place, and maintained until the product is dry. The shrinkage and its follow-up is readily seen in a multiple-platen press to considerably exceed the expansion incident to the pressure reduction.

After the moisture has been reduced, for example reduced down to around 5% or less, the pressure can be increased if desired, particularly 25 with the higher gravity board, up to the initial extra high pressure or higher as desired, as for example 1000 pounds per square inch, to get the benefit of high pressures in the final stages of the operation but the lower pressure may be carried through until the board is finished. So long as scorching is avoided, the final pressure and temperature application may be kept up, and applied to the board for a time after it is dry. The steam valves to the platens can be closed and 30 the boards removed as soon as dry and the platens allowed to cool somewhat before the next pressure application, though the heating steam may be applied uninterruptedly if desired.

We claim:

40 1. Process of making hard products, such as board and the like, of a body of ligno-cellulose fiber containing a sufficiently high proportion of non-cellulose to produce thorough bonding and containing 25% or over of water, which comprises 45 pressing same in a hot press with wire mesh between the fiber body and a press platen with initial application of relatively high pressure, and then reducing the pressure, and continuing the drying of the product in place between the 50 heated platens under pressure considerably lower than that initially applied, but not, however, below about 60 lbs. per square inch.

2. Process as in claim 1, in which the initial pressure is several times the lower pressure used 55 later.

3. Process as in claim 1, in which the body of fiber contains 50% or over of water.

4. Process as in claim 1, but in which the pressure is again raised prior to completing the board 60 and after the moisture has been reduced to about 5% or under.

5. Process as in claim 1, in which the initial pressure is approximately 400-500 pounds per square inch, applied for approximately 1 minute, followed by pressure of about 100-125 pounds per square inch applied for approximately 10 minutes, and the hardboard produced is of specific gravity approximately 1-1.05.

6. Process as in claim 1, in which the initial 70 pressure is approximately 200 pounds per square inch, applied for approximately 1 minute, followed by pressure of about 60 pounds per square inch applied for approximately 20 minutes, and the hardboard produced is of specific gravity approximately .9.

7. Process of making hard products such as board and the like, of a body of ligno-cellulose fiber containing a sufficiently high proportion of non-cellulose to produce thorough bonding and containing 25% or over of water, which comprises 5 pressing same in a hot press with moisture escape conduits between the fiber body and a press platen with initial application of relatively high pressure, and then, without the pressure having ever been completely released, completing 10 the drying of the product in place between the heated press platens, and under much lower pressure.

8. Process of making a hard board or like product which comprises nearly drying under 15 moderate pressure of approximately 60-125 pounds per square inch after initially applying pressure several times as high to a body of ligno-cellulose containing 25% or over of water and containing plenty of the noncellulose thereof to 20 insure thorough coalescing and bonding, and after the board is nearly dried, completing the drying under a reapplication of elevated pressure.

9. Process as in claim 8, in which temperature of 430° F. or over is applied to the board during 25 the application of pressure.

10. Process as in claim 8, in which temperature of 430-550° F. is applied to the board during the application of pressure.

11. Process of making hard products, such as 30 board and the like, of a body of ligno-cellulose fiber containing a sufficiently high proportion of non-cellulose to produce thorough bonding and containing 25% or over of water, which comprises 35 pressing same in a hot press at a temperature of over 430° F. and preferably about 450-550° F. with wire mesh between the fiber body and a press platen with initial application of relatively high pressure, and then, without the pressure having ever been completely released, completing 40 the drying under much lower pressure whereby to make a product of high dry and wet strength and substantially free from surface defects in a single press-drying operation.

12. Process of making hard products, such as 45 board and the like, of a body of ligno-cellulose fiber containing a sufficiently high proportion of non-cellulose to produce thorough bonding and containing 25% or over of water, which comprises 50 pressing same in a hot press at a temperature of over 430° F. and preferably about 450-550° F. with wire mesh between the fiber body and a press platen making initial application of relatively high pressure, and then materially reducing the pressure without, however, completely releasing the pressure and completing the drying of the product between the heated press platens at the reduced pressure, whereby to make a hard product of high dry and wet strength substantially 60 free from surface defects in a single press-drying operation.

13. The process of making hard products, such as board and the like, of a body of ligno-cellulose fiber containing a sufficiently high proportion of 65 non-cellulose to produce thorough bonding and containing 25% or over of water, which comprises pressing same in a hot press with wire mesh between the fiber body and a press platen with initial application of relatively high pressure where- 70 by to drive water out especially from that part of the body of fiber adjacent said wire mesh; redistributing the remaining water content throughout the entire fiber body by lowering the pressure without completely releasing same, and 75

completing the drying while maintaining a pressure on said body of the lowered order of pressure, and following up the pressure application as shrinkage occurs and until the board is dry, whereby to make a hard, dense board of high dry and wet strength and substantially free from surface defects in a single press-drying operation.

14. The process of making hard products, such as board and the like, of a body of ligno-cellulose fiber containing a sufficiently high proportion of non-cellulose to produce thorough bonding and containing 25% or over of water, which comprises pressing same in a hot press at a temperature of over 430° F. and preferably about 450°-550° F. with wire mesh between the fiber body and a press platen with initial application of relatively high pressure whereby to drive water out especially from that part of the body of fiber adjacent said wire mesh; redistributing the remaining water content throughout the entire fiber body by lowering the pressure without completely releasing same, and completing the drying while maintaining a pressure on said body of the lowered order of pressure, whereby to make a hard, dense board of high dry and wet strength and substantially free from surface defects in a single press-drying operation.

15. Process of making products, such as board and the like, of a body of ligno-cellulose fiber containing a sufficiently high proportion of non-

cellulose to produce thorough bonding and containing 25% or over of water, which comprises subjecting said fiber body to a single-step press drying operation in a hot press with wire mesh between the fiber body and a press platen comprising making initial application of relatively high pressure, and then without the pressure having ever been released, completing the drying under much lower pressure, and following up such pressure application as shrinkage occurs and until the board is dry, whereby to make a hard product of high dry and wet strength, substantially free from surface defects.

16. Process as in claim 15 wherein the temperature applied in the hot-pressing is over 430° F. and preferably about 450-550° F.

17. Process of making hard products such as board and the like, of a body of ligno-cellulose fiber containing a sufficiently high proportion of non-cellulose to produce thorough bonding and containing 25% or over of water, which comprises pressing same in a hot press at a temperature of about 350°-430° F. with moisture escape conduits between the fiber body and a press platen with initial application of relatively high pressure, and then, without the pressure having ever been completely released, completing the drying of the product in place between the heated press platens, and under much lower pressure.

WILLIAM H. MASON.

CHARLES H. WESTPHALEN.

30